

L. A. JEFFS.

PROCESS FOR MAKING ALLOYS OF PHOSPHORUS.

APPLICATION FILED NOV. 13, 1917.

1,268,849.

Patented June 11, 1918.



Inventor

L. A. Jeffs, by

G. W. Schuberspoon

Attorney

# UNITED STATES PATENT OFFICE.

LEWIS A. JEFFS, OF SALT LAKE CITY, UTAH.

## PROCESS FOR MAKING ALLOYS OF PHOSPHORUS.

1,268,849.

Specification of Letters Patent. Patented June 11, 1918.

Application filed November 13, 1917. Serial No. 201,780.

To all whom it may concern:

Be it known that I, LEWIS A. JEFFS, a citizen of the United States, residing at Salt Lake City, in the county of Salt Lake and State of Utah, have invented certain new and useful Improvements in Processes of Making Alloys of Phosphorus; and I do hereby declare the following to be a full, clear, and exact description of the invention, such as will enable others skilled in the art to which appertains to make and use the same.

This invention relates to a process of producing alloys of phosphorus, especially of copper and phosphorus, or cupro-phos, and has for its object to provide a method which will be more expeditious and less expensive than those heretofore proposed.

With these and other objects in view the invention consists in the novel steps and combinations of steps constituting the process, all as will be more fully hereinafter disclosed and particularly pointed out in the claims.

Referring to the accompanying drawing, forming a part of this specification, in which the figure is a diagrammatic sectional view of a type of furnace especially adapted for practising the invention, 1 indicates any suitable hearth, 2 an exit for the alloy of metal and phosphorus, 3 a molten pool of said alloy, 4 a slag exit, 5 any suitable lining for the walls 6 of the furnace, 7 any suitable form of electrodes provided with the connections 8, 9 an exit or downcomer for the evolved gases, 10 the usual bell for closing the top 11 of the furnace, and 12 the charge made up of phosphate rock, the metal, or material carrying the metal, it is desired to alloy with the phosphorus, and carbon in suitable proportions.

It is well known that phosphate rock will give up its phosphorus either in the form of oxids, or as elemental phosphorus, according to the temperature to which it may be subjected, and also according to the amount of carbon and oxygen present in the fusion zone. It is further well known that if one employs a blast furnace, maintains a localized fusion zone at a very high tempera-

ture using preheated air, and also maintains an excess of carbon in the fusion zone, the alloying of phosphorus with any molten iron present in the charge to form ferro-phos, will be facilitated. In such a process 55 it is found that the preheating of the downcoming charge owing to the upward passage of the evolved gases therethrough greatly promotes the liberation of the phosphorus and its entry into the iron. 60

In other words, it is well known that a blast type of furnace lends itself to both efficiency and economy in the making of ferro-phos of a high content of phosphorus, and in this invention, I closely follow in the 65 furnace illustrated in the drawings, the shape of the ordinary blast furnace, except the stack is much shorter, and no twyers are provided.

If cupro-phos is to be produced, I make 70 up a suitable balance charge 12 of a fluxing material, phosphate rock, metallic copper, copper matte, or an oxidized copper ore, and carbon. A sulfid copper ore would not be suitable, although the sulfur content of 75 the matte is not seriously detrimental. The carbon in the charge should be in such excess of that required by theory as to always insure an excess of incandescent carbon in the fusion zone, or space 14 between and 80 around the electrodes.

The reason for this said excess of incandescent carbon resides in the fact that, unless the temperature of the fusion zone is very high indeed, the phosphorus will be 85 liberated in the form of oxids, a form in which it will not enter the metal; and therefore, unless an ample supply of incandescent carbon is present at the point of liberation to reduce these said oxids to elemental 90 phosphorus, they will escape with the exit gases. To insure that substantially all of the liberated combined phosphorus is reduced to the elemental condition, I sometimes provide the carbon in such quantities that it is 95 40% in excess of theoretical requirements.

The copper being melted and reduced if in a combined state at relatively low temperatures, the elemental phosphorus will enter it at points in the charge much higher 100

2  
than those at which the phosphorus oxids are liberated, and therefore, said oxids will naturally rise up through the excess of incandescent carbon in the fusion zone and 5 be reduced, before reaching the molten copper in the upper regions of said zone.

As the phosphorus alloys with the copper in the manner just disclosed, the cupro-phos thus formed will trickle down through the 10 charge, meeting ascending phosphorus on its way, and finally collect in the pool 3.

The incandescent exit gases containing more or less  $P_2O_5$  and elemental phosphorus will pass up through the interstices of the 15 charge, preheating the latter as it descends, and will be collected in the downcomer 9, whence they will be subjected to a scrubbing action for the recovery of their values, or otherwise treated as desired.

20 The slag floats on the pool 3, and is tapped off from time to time through the exit 4, and the cupro-phos at the exit 2.

The maintenance of an excess of incandescent carbon in the fusion zone by the aid 25 of an electric current instead of by a hot blast of air enables me to regulate the temperature of said zone over wide ranges and to maintain it substantially constant, and therefore, to produce greater quantities of 30 elemental phosphorus for the impregnation of the copper and a more uniform content of phosphorus in the alloy than would be possible with a hot blast.

It results from this that I am enabled to 35 produce directly from the rock much higher contents of phosphorus in alloys of copper, iron, etc., than would be possible in a blast furnace, and further, by properly proportioning the metal to the phosphorus and 40 carbon in the charge, I am enabled to produce any desired richness of oxids of phosphorus and of elemental phosphorus in the exit gases.

In fact, by employing a relatively small 45 quantity of copper or iron, and a great excess of phosphate rock and carbon, I am enabled to make the exit gases so rich in phosphorus as to warrant its recovery as the principal product of the process. Of course, 50 if  $P_2O_5$  is desired, the exit gases can be readily burned and this product recovered.

It will thus be seen that by substituting an electric current for a hot blast in a blast 55 type of furnace, I am enabled to use a minimum of carbon, for although the latter is greatly in excess of that theoretically required, yet, no free oxygen is admitted to consume the same, and therefore, only a quantity in excess of that necessary to reduce 60 the phosphorus and other oxids present is required. In fact, this said carbon accumulates above the slag, in the fusion zone, and after the furnace is running its proportion in the charge can be reduced. It 65 will be further observed that by employing

a furnace having the shape shown, the charge descends gradually and evenly with little tendency to stick, and by employing electric heat instead of a hot blast combustion, the reaction zone is more localized; no molten 70 pool is required to keep the furnace from running cold; a reacting concentrated gas phase is produced undiluted with nitrogen, and therefore, the metal is more readily impregnated; and the incandescent carbon instead of carbon monoxid may be relied upon 75 to reduce the oxidized ore as well as the oxid of phosphorus, thus reducing the  $CO$  and  $CO_2$  gases leaving the stack, to a minimum. 80

The amperage, voltage, proportions of rock to carbon, proportions and kind of metal in the charge, etc., of course, will vary according to the materials at hand and the purpose of the operator, but these data will 85 be readily ascertained by the skilled furnace man.

It is obvious that those skilled in the art may vary the details of the process without departing from the spirit of the invention, 90 and therefore, I do not wish to be limited to the above disclosure except as may be required by the claims.

What I claim is:—

1. The process of making an alloy of a 95 metal and phosphorus in an electric furnace which consists in providing a charge containing phosphate rock and carbon; adding to said charge a material adapted to supply said metal; passing a current of electricity 100 through a portion of said charge to produce said metal in a fused condition and sufficient to evolve oxids of phosphorus in a gaseous condition while providing a localized fusion zone; and maintaining an excess of 105 incandescent carbon in said zone, substantially as described.

2. The process of making an alloy of a 110 metal and phosphorus in an electric furnace which consists in providing a charge of phosphate rock, fluxing material and carbon in excess; adding to said charge a material capable of supplying said metal in a fused state above the fusion zone when said rock is being decomposed; passing a current of 115 electricity through a portion of said charge to provide a localized fusion zone and of a sufficient strength to cause oxids of phosphorus to be evolved from said rock; and maintaining in said charge an excess of free 120 incandescent carbon to reduce said oxids of phosphorus, substantially as described.

3. The process of making an alloy of 125 phosphorus and copper in an electric furnace which consists in providing a charge of phosphate rock and carbon; adding to said charge a material capable of supplying metallic copper in a fused state above the fusion zone while said rock is being decomposed; passing a current through a portion 130

of said charge to provide a localized fusion zone and of a sufficient strength to produce oxids of phosphorus from said rock; and maintaining an excess of free incandescent 5 carbon in said zone to reduce said oxids as fast as they are formed, substantially as described.

In testimony whereof I affix my signature, in presence of two witnesses.

LEWIS A. JEFFS.

Witnesses:

E. J. HAWKE,  
ROBERT E. MARK.